

1

2,739,057

## ALLOY STEEL OF HIGH EXPANSION COEFFICIENT

Peter Payson, New York, N. Y., assignor to Crucible Steel Company of America, New York, N. Y., a corporation of New Jersey

No Drawing. Continuation of application Serial No. 201,870, December 20, 1950. This application October 24, 1952, Serial No. 316,803

10 Claims. (Cl. 75—123)

This invention pertains to alloy steels which are characterized in possessing relatively high coefficients of expansion.

This application is a continuation of my copending application Serial No. 201,870, filed December 20, 1950, now abandoned, and entitled "Alloy Steel of High Expansion Coefficient."

It is the object of the invention to provide an alloy steel having a higher coefficient of expansion over the range of room temperature to 600° F., than is now available in known steels. A steel of this character is required for use as high strength bolts, screws, tie rods, and other parts in assemblies made with aluminum pieces, in order that the fit between the steel and the aluminum be maintained as tight as possible. As is well known, aluminum and its alloys have a much higher coefficient of expansion for the range 70° to 600° than steel, namely about  $15 \times 10^{-6}$  inch per inch per degree F., as against  $7.5 \times 10^{-6}$  for ordinary carbon or ferritic steels, and about 10.0 to  $10.5 \times 10^{-6}$  for the austenitic stainless steels.

There has been available for some time a special composition of steel of analysis,

| Percent C | Percent Mn | Percent Ni | Percent Cr | Percent Mo | Bal. |
|-----------|------------|------------|------------|------------|------|
| .50       | 3.5        | 11.0       | 3.0        |            |      |
| .60       | 5.5        | 14.0       | 5.0        | .50 max.   | Fe   |

covered by Aeronautical Specification 5624A, which has the highest coefficient of expansion of any steel so far produced, namely, about 11.0 to  $11.2 \times 10^{-6}$ . However, this expansion value is still far short of that of aluminum and its alloys, and there is a demand for a steel with a higher expansion value.

Another object of this invention is to provide a high expansion steel of lower alloy content than the high expansion steels now being used. This is a factor of strategic as well as of economic importance.

It is well known that austenitic steels have higher expansion values than steels containing the transformation products of austenite, that is, ferrite, pearlite, bainite, or martensite. Also it is well known that some compositions of austenite have expansion values different from those of others as shown in Table I, below, taken from data published in U. S. Department of Commerce, Circular C447, "Mechanical Properties of Metals and Alloys."

TABLE I

Expansion values of some known austenitic steels

| No.  | Analysis, Percent |     |      |      |      | Bal.   | Expansion Coefficient for the Range 70° to 750° F. in. per in. $\times 10^{-6}$ per ° F. |      |
|------|-------------------|-----|------|------|------|--------|------------------------------------------------------------------------------------------|------|
|      | C                 | Mn  | Si   | Ni   | Cr   |        |                                                                                          |      |
| 2446 | .40               |     |      | 13   | 13   | 2.5 W  | Fe                                                                                       | 9.8  |
| 2449 | .06               | .36 | .28  | 9.6  | 17.7 | Fe     | Fe                                                                                       | 10.1 |
| 2474 | .39               | .74 | 1.12 | 20.2 | 7.9  | .22 Cu | Fe                                                                                       | 10.5 |
| 2481 | .39               |     |      | 36.1 |      | .39 Cu | Fe                                                                                       | 3.5  |
| 2483 | .42               | .71 | 1.03 | 36.0 | 16.4 | Fe     | Fe                                                                                       | 8.5  |

2

It is clear from Table I that none of these steels has a coefficient as high as that of the AMS 5624A analysis given above.

Now I have discovered that a steel of relatively low nickel content, that is, about 6 to 13% with enough carbon and manganese in it to stabilize the austenite of the steel, and containing practically no chromium, has a higher coefficient than steel of the AMS 5624A analysis, and so far as is known, higher than any other steel previously known.

The steel of my invention contains according to the broad range of analysis, about .40 to 1.00% carbon, about 3.0 to 13.0% manganese and about 6 to 13% nickel, the sum of nickel and manganese being preferably at least 11%, and the balance being substantially all iron with usual impurities, although the steel may include optional additions of up to about 2.0% in aggregate of one or more of the elements Si, V, Mo and W, and a maximum of 0.5% Cr. In the annealed condition, that is, as air cooled from about 2100° F., this steel has a coefficient of expansion of  $12.0 \times 10^{-6}$  inch per inch per degree F. for the range 70° to 600° F. Within the limits of composition, just given, the value of the expansion coefficient of the steel is practically unaffected by composition changes as may be seen in Table II.

TABLE II

Steels of this invention which as annealed have a coefficient of expansion value over the range from 70° to 600° F. of about  $12.0 \times 10^{-6}$  inch per inch per degree F.

| 35   | Bar | Analysis, Percent |      |     |      |      |      |
|------|-----|-------------------|------|-----|------|------|------|
|      |     | C                 | Mn   | Si  | Ni   | Cr   | Bal. |
| 2797 |     | .55               | 5.2  | .11 | 6.1  | 0.09 | Fe   |
| 2798 |     | .69               | 9.1  | .11 | 6.1  | 0.02 | Fe   |
| 2799 |     | .68               | 12.9 | .13 | 6.0  | 0.02 | Fe   |
| 2800 |     | .59               | 5.3  | .31 | 8.9  | 0.05 | Fe   |
| 2801 |     | .57               | 8.8  | .33 | 8.8  | 0.07 | Fe   |
| 2802 |     | .66               | 12.8 | .18 | 9.0  | 0.02 | Fe   |
| 2803 |     | .50               | 4.9  | .05 | 11.9 | 0.03 | Fe   |
| 2804 |     | .69               | 9.2  | .13 | 13.0 | 0.01 | Fe   |
| 2839 |     | .61               | 4.8  | .71 | 12.1 | 0.20 | Fe   |
| 2805 |     | .73               | 13.6 | .16 | 12.9 | 0.00 | Fe   |

When the nickel content of the steel is over about 13%, or when the chromium content of the steel is high, that is, over about 0.5%, the expansion coefficient is less than  $12.0 \times 10^{-6}$  as is shown in Table III.

TABLE III

Effects of high nickel and chromium on the expansion coefficient of austenitic steels

[All samples tested as annealed, i. e., air cooled from 2100° F.]

| 55   | Bar | Analysis, Percent |     |     |      |     |      | Expansion Coefficient for range 70° to 600° F. in. per in. $\times 10^{-6}$ per ° F. |
|------|-----|-------------------|-----|-----|------|-----|------|--------------------------------------------------------------------------------------|
|      |     | C                 | Mn  | Si  | Ni   | Cr  | Bal. |                                                                                      |
| 2639 |     | .61               | 4.8 | .71 | 12.1 | 0.2 | Fe   | 12.0                                                                                 |
| 2408 |     | .58               | 5.0 | .53 | 13.8 | 4.9 | Fe   | 11.1                                                                                 |
| 2642 |     | .58               | 5.1 | .61 | 15.8 | 0.1 | Fe   | 11.7                                                                                 |
| 2644 |     | .62               | 4.9 | .59 | 16.1 | 3.4 | Fe   | 11.0                                                                                 |

It is clear from these data and those of Table II, that chromium has a marked effect on the expansion coefficient, causing it to be decreased appreciably; and that nickel upwards of about 13% causes the steel to have a lower expansion coefficient than a steel containing nickel within the range of the present invention, i. e., 6 to 13%.

Since the steel of this invention is austenitic and therefore cannot be hardened except by cold working; and

since it may be desired that the steel be cold worked in order to strengthen it, I balance the composition of the steel so that it is stably austenitic even after it is cold worked appreciably, for example, to a hardness of about Rockwell C 28 to 38.

If the austenite of the steel transforms to an appreciable degree because of cold working, as would be indicated by the fact that the steel becomes appreciably magnetic, the coefficient of the steel decreases. This is shown by the comparative data of the following Table IV.

TABLE IV

*Effect of composition on the expansion coefficient of austenitic steels after cold working*

[Samples tested both as annealed, i. e., air cooled from 2,100° F., and as cold worked about 22% from the annealed condition.]

| Bar  | Analysis, percent |     |     |     | Condition   | Hardness, Rockwell | Magnetic Suscept. <sup>1</sup> | Expansion Coefficient from 70° to 600° F. in. per in. $\times 10^{-6}$ per ° F. |
|------|-------------------|-----|-----|-----|-------------|--------------------|--------------------------------|---------------------------------------------------------------------------------|
|      | C                 | Mn  | Si  | Ni  |             |                    |                                |                                                                                 |
| 2797 | .55               | 5.2 | .11 | 6.1 | Annealed    | B76                | N. M.                          | 12.0                                                                            |
| 2797 | .55               | 5.2 | .11 | 6.1 | Cold Worked | C36                | M.                             | 11.6                                                                            |
| 2798 | .69               | 9.1 | .11 | 6.1 | Annealed    | B31                | N. M.                          | 12.0                                                                            |
| 2798 | .69               | 9.1 | .11 | 6.1 | Cold Worked | C35                | VSM                            | 12.0                                                                            |

<sup>1</sup> N. M.—non magnetic; M.—magnetic; VSM—very slightly magnetic.

On the basis of these data a steel in accordance with the invention but of higher alloy content than the minimum, should be used whenever the steel is to be cold worked or is to be subjected to very low temperatures which might tend to cause appreciable transformation of the austenite.

The preferred range of composition of the steel of this invention is: .50 to .70% carbon; 5.0 to 9.0% manganese; up to 1.0% silicon; up to 0.5% chromium; 6.0 to 10.0% nickel; up to 2.0% in aggregate of other elements not detrimental to the high expansion properties of the steel; balance iron.

Especially useful analyses are those of Table V below.

TABLE V  
Analysis, percent

|   | Analysis, Percent |     |      |      |                             |
|---|-------------------|-----|------|------|-----------------------------|
|   | C                 | Mn  | Si   | Ni   | Balance                     |
| 1 | .55               | 8.0 | .20  | 5.0  | Iron with usual impurities. |
|   | .65               | 9.0 | 1.00 | 6.0  |                             |
| 2 | .55               | 7.0 | .20  | 7.0  | Do.                         |
|   | .65               | 8.0 | 1.00 | 8.0  |                             |
| 3 | .55               | 5.0 | .20  | 9.0  | Do.                         |
|   | .65               | 6.0 | 1.00 | 10.0 |                             |
| 4 | .55               | 4.0 | .20  | 11.0 | Do.                         |
|   | .65               | 5.0 | 1.00 | 12.0 |                             |

I claim:

1. A forgeable, austenitic alloy steel, characterized in having a coefficient of expansion of at least  $11.8 \times 10^{-6}$  inch per inch per degree F., over the temperature range of about 70° to 600° F., said steel containing: about 0.5 to 0.7% carbon; about 6 to 10% nickel; about 5 to 9% manganese; up to about 0.5 chromium; up to about 1% silicon; up to about 2% in aggregate of other elements which do not impair the high coefficient of expansion of the steel; and the balance iron.

2. A forgeable, austenitic alloy steel, characterized in having a coefficient of expansion of at least  $11.8 \times 10^{-6}$  inch per inch per degree F., over the temperature range of about 70° to 600° F., said steel containing: about 0.5 to 0.7% carbon; about 6 to 10% nickel; about 5 to 9% manganese; up to 1.0% silicon; and the balance iron.

3. A fastening element for uniting structural com-

ponents having high expansion coefficients, said fastening element being made of a work hardened austenitic alloy steel having a hardness of at least Rockwell C 28, and having a coefficient of expansion at least  $11.8 \times 10^{-6}$  inch per inch per degree F., said steel containing: about 0.4 to 1.0% carbon; about 6 to 13% nickel, and about 3 to 14% manganese, the sum of nickel and manganese being at least 11%; up to about 0.5% chromium; up to about 2% in aggregate of at least one element selected from the group consisting of silicon, vanadium, tungsten

and molybdenum; and the balance substantially all iron.

4. A fastening element for uniting structural components having high expansion coefficients, said fastening element being made of a work hardened austenitic alloy steel having a hardness of at least Rockwell C 28, and having a coefficient of expansion of at least  $11.8 \times 10^{-6}$  inch per inch per degree F., said steel containing: about 0.5 to 0.7% carbon; about 6 to 10% nickel; about 5 to 9% manganese; up to about 0.5% chromium; up to about 1% silicon; up to about 2% in aggregate of other elements which do not impair the high coefficient of expansion of the steel; and the balance iron.

5. A fastening element for uniting structural components having high expansion coefficients, said fastening element being made of a work hardened austenitic alloy steel having a hardness of at least Rockwell C 28, and having a coefficient of expansion of at least  $11.8 \times 10^{-6}$  inch per inch per degree F., said steel containing: about 0.4 to 1.0% carbon; about 6 to 13% nickel, and about 3 to 14% manganese, the sum of nickel and manganese being at least 11%; up to 1.0% silicon; and the balance iron.

6. A fastening element for uniting structural components having high expansion coefficients, said fastening element being made of a work hardened austenitic alloy steel having a coefficient of expansion of at least  $11.8 \times 10^{-6}$  inch per inch per degree F., said steel containing: about 0.5 to 0.7% carbon; about 6 to 10% nickel; about 5 to 9% manganese; up to 1.0% silicon; and the balance iron.

7. A forgeable, austenitic alloy steel, characterized in having a coefficient of expansion of at least  $11.8 \times 10^{-6}$  inch per inch per degree F., over the temperature range of about 70° to 600° F., said steel containing: about 0.55 to 0.65% carbon; about 5 to 6% nickel; about 8 to 9% manganese; about .20 to 1% silicon; and the balance iron.

8. A forgeable, austenitic alloy steel, characterized in having a coefficient of expansion of at least  $11.8 \times 10^{-6}$  inch per inch per degree F., over the temperature range of about 70° to 600° F., said steel containing: about 0.55 to 0.65% carbon; about 7 to 8% nickel; about 7 to 8% manganese; about 0.20 to 1% silicon; and the balance iron.

9. A forgeable, austenitic alloy steel, characterized in having a coefficient of expansion of at least  $11.8 \times 10^{-6}$  inch per inch per degree F., over the temperature range of about 70° to 600° F., said steel containing: about

0.55 to 0.65% carbon; about 9 to 10% nickel; about 5 to 6% manganese; about 0.20 to 1% silicon; and the balance iron.

10. A forgeable, austenitic alloy steel, characterized in having a coefficient of expansion of at least  $11.8 \times 10^{-6}$  inch per inch per degree F., over the temperature range of about 70° to 600° F., said steel containing: about 0.55 to 0.65% carbon; about 11 to 12% nickel; about 4 to 5% manganese; about 0.20 to 1% silicon; and the balance iron.

References Cited in the file of this patent

UNITED STATES PATENTS

|           |           |               |    |
|-----------|-----------|---------------|----|
| 452,494   | Fessenden | May 19, 1891  | 15 |
| 1,843,903 | Scott     | Feb. 2, 1932  |    |
| 1,902,589 | Scott     | Mar. 21, 1933 |    |
| 2,217,422 | Scott     | Oct. 8, 1940  |    |
| 2,220,690 | Stupakoff | Nov. 5, 1940  |    |

FOREIGN PATENTS

7,422 Great Britain \_\_\_\_\_ Apr. 3, 1897  
of 1896

OTHER REFERENCES

Metal Progress, November 1931, pages 69 to 72.

The Book of Stainless Steels, 2nd edition, Thum, published 1935 by the A. S. M., Cleveland, Ohio; page 340.

Alloys of Iron and Chromium, High Chromium, vol. 2, page 289. Edited 1940 by Kinzel and Franks.

Cold Working of Metals, page 2. Published in 1949, by the American Society for Metals, Cleveland, Ohio.

Symposium on "Effect of Temperature on the Properties of Metals," published jointly (1931) by the ASTM and ASME (New York); pages 693 and 694 are particularly pertinent in paper on "Thermal Expansion of Metals" by Mochel.

Revue de Metallurgie, Memoires, Tome 2, 1905, pages 827-833.